

3,454,625

NOVEL QUATERNARY AMMONIUM CARBAMATE  
ANTISTATIC AGENTSFred S. Eiseman, Jr., Maplewood, and Leslie M. Schenck,  
Mountainside, N.J., assignors to GAF Corporation,  
New York, N.Y., a corporation of Delaware

No Drawing. Filed Apr. 3, 1967, Ser. No. 627,859

Int. Cl. C07c 125/06, 87/30; D06m 13/46

U.S. Cl. 260—482

6 Claims

## ABSTRACT OF THE DISCLOSURE

Antistatic agents of the formula:



wherein R is an alkyl or alkaryl radical containing at least 7 carbon atoms; X is hydrogen, methyl, or ethyl; n is an integer from 1 to 10; R<sub>1</sub> and R<sub>2</sub> are alkyl or hydroxy alkyl radicals of 1-3 carbon atoms; R is a hydroxyalkyl radical of from 1-4 carbon atoms; and Y is an anion.

These antistatic agents, particularly useful for synthetic fibers, are prepared by condensing an alkyl or aryl polyalkyleneoxy chlorocarbonate with a substituted alkyl diamine with subsequent acidification and alkoxylation to produce the quaternary compound, the chlorocarbonate being prepared by the reaction of the corresponding hydroxy compound with phosgene.

The present invention relates to new and useful compositions of matter which function as antistatic agents when coated on synthetic and natural fibers, e.g., polyester fibers, acetate rayons, wool, polyolefins and the like, and to the method for their preparation. More particularly, the present invention relates to substituted carbamates exhibiting antistatic properties which are prepared by the condensation of alkyl and aryl polyalkyleneoxy chlorocarbonates with a substituted alkyl diamine followed by acidification and alkoxylation.

The commercial importance of the synthetic fibers industry has greatly emphasized the importance of antistatic agents and finishes since synthetic fibers, e.g., polyester fibers, acrylics, vinyls, etc., are notorious static electricity generators. While other fibers, e.g., cotton or viscose, do not generate the static electricity to any great extent under normal humidity conditions, and fibers such as acetate, rayon, and wool are only moderate generators, necessitating only some precautionary measures in the processing mill, e.g., a controlled high humidity, synthetic fibers such as mentioned above are not easily treated to control static electricity buildup.

While several non-durable finishes have been proposed which are moderately effective in eliminating static buildup on these synthetic fibers, few have been proposed which are completely satisfactory durable antistats. Most finishes employed to eliminate static buildup on synthetic fibers fall into the category of true surfactants although there is no really distinct similarity or correlation between surface activity and antistatic action.

In general, antistatic agents function in two ways, both of which improve the electrical conductivity of the fiber surface. Such antistatic agents are either reasonably good conductors of electricity themselves, or they are hygroscopic and help concentrate atmospheric moisture on the fibers.

The majority of antistatic agents fall into one of the following three categories: (1) polyhydroxy and polyethylenoxy non-ionic compounds; (2) cationic, or neutral

nitrogenous compounds with a hydrophobic moiety in their structure; (3) long-chain phosphates, phosphonates, or other oxygenated phosphorus derivatives. Additional types include sulfonated oils and ester emulsions, and other fiber lubricant emulsions which depend on the particular emulsifying agent used for their antistatic effect.

Long chain quaternary ammonium salts have a marked antistatic action and are widely used in this capacity. These quaternaries, in common with numerous antistatic finishes, are frequently used in combination with auxiliary agents which may themselves be antistats, or serve the secondary purpose of binding the finish to the fiber, as disclosed in U.S. 2,463,282. The water-insoluble salts of higher amines, together with polystyrene sulfonates, are described in U.S. 2,700,001 as nylon antistats. The use of phosphorus compounds in antistatic capacities is given in U.S. 2,575,382, 2,575,399, and 2,676,122. Hygroscopic salts, such as cyclohexylamine lactate, are disclosed in German Patent 840,694, while the use of polyethoxylated fatty acids and alcohols as antistatic agents for polypropylenes as well as fibers, is reported in U.S. 2,525,691.

In accordance with the present invention, it has now been found that certain compounds which incorporate a carbamate structure within the molecule, and more specifically, those derived from the chlorocarbonate of an alkoxyated primary or secondary alcohol, or alkylphenol, and a dialkylaminopropylamine, show excellent antistatic properties when applied to synthetic fibers. These novel carbamates impart not only the antistatic activity associated with both an amide linkage and that imparted by a quaternary configuration, but also the desirable antistat characteristics of a polyalkoxylated hydrophobe. Unexpectedly the combination of these chemical functions within the carbamate molecular structure provides an enhancement lacking through the simple admixture of non-ionic and amide type antistatic agents.

It is, therefore, a principal object of the present invention to prepare new and useful substituted carbamate antistatic agents.

A further object of the present invention comprises antistatic agents of enhanced effectiveness, which antistatic agents contain an amide linkage and a polyalkoxylated hydrophobe.

Yet a further object of the present invention comprises new and useful substituted carbamate antistatic agents derived from the chlorocarbonate of an alkoxyated primary or secondary alcohol or alkylphenol and a substituted alkyl diamine.

Still a further object of the present invention comprises a process for preparing new and useful antistatic agents which process comprises condensing an alkyl or aryl polyalkyleneoxy chlorocarbonate with an alkyl diamine followed by acidification and alkoxylation.

Still further objects of the present invention will become more apparent from the following more detailed description of the invention.

The new and useful antistatic agents of the present invention correspond to the general formula:



wherein R is an alkyl or alkaryl radical containing at least 7 carbon atoms,

X is hydrogen, methyl, or ethyl;

n is an integer from 1 to 10;

R<sub>1</sub> and R<sub>2</sub> are alkyl or hydroxyalkyl radicals of 1-3 carbon atoms;

R<sub>3</sub> is a hydroxyalkyl radical of from 1-4 carbon atoms; and

Y is an anion.

Exemplary alkyl or alkaryl radicals for R include: heptyl, octyl, nonyl, decyl, undecyl, dodecyl, tridecyl, hexadecyl, octadecyl, nonadecyl, eicosyl, docosyl, pentacosyl, etc., methylphenyl, ethylphenyl, butylphenyl, hexylphenyl, octylphenyl, nonylphenyl, decylphenyl, dodecylphenyl, pentadecylphenyl, octadecylphenyl, nondecylphenyl, etc.

Exemplary alkyl and hydroxylalkyl radicals for  $R_1$  and  $R_2$  include: methyl, ethyl, propyl, isopropyl, hydroxymethyl, hydroxyethyl, hydroxypropyl dihydroxypropyl, etc.

Exemplary hydroxyalkyl radicals for  $R_3$  include; hydroxymethyl, hydroxyethyl, hydroxypropyl, hydroxybutyl, dihydroxypropyl, dihydroxybutyl, etc.

Exemplary anions for Y include: halides, chloride, bromide, iodide, phosphates, nitrates, sulfates, and the like.

The new and useful antistatic agents of the present invention are prepared by condensing an alkyl or alkaryl polyalkylenoxy chlorocarbonate with a substituted alkyl-diamine followed by acidification and alkoxylation.

The alkyl or alkaryl polyalkylenoxy chlorocarbonate is prepared by reacting phosgene with a polyalkylene-oxylated aliphatic alcohol or alkylphenol under ambient conditions, in accordance with the following reaction:



In general, a substantially equivalent amount of the reactants is employed and the reaction is carried out by bubbling phosgene under the surface of the polyalkylene-oxylated aliphatic alcohol or alkylphenol until substantially all of the hydroxyl content of the reactants is converted into the chlorocarbonate as determined by infrared analysis or other suitable means.

The polyalkyleneoxylated aliphatic alcohol or alkylphenol is prepared by any conventional procedure so as to incorporate 1 to 10 moles of alkylene oxide, e.g., ethylene oxide, propylene oxide, or butylene oxide per mole of aliphatic alcohol or alkylphenol. The alkyl or alkaryl polyalkyleneoxy chlorocarbonate prepared in Reaction I is further reacted with a substantially equivalent amount of gamma dialkyl or dialkanol aminopropylamine to produce a substituted amide in accordance with the following reaction:



The substituted amide produced in Reaction II is quaternized by reaction with an alkylene oxide or hydroxy-substituted alkylene oxide in the presence of an inorganic acid. Such a reaction is represented as follows:



Reaction III above can be more precisely broken down into two separate reactions as follows:



5 and  
IIIb



15 In the Reactions I, II, III, III $a$  and III $b$  above, R, R<sub>1</sub>, R<sub>2</sub>, R<sub>3</sub>, X, Y and  $n$  are as previously defined.

In the preferred synthesis, a commercial straight chain aliphatic alcohol admixture comprising approximately 5% C<sub>11</sub>, 25% C<sub>12</sub>, 30% C<sub>13</sub>, 30% C<sub>14</sub> and 10% C<sub>15</sub> is reacted 20 with an alkylene oxide using an alkaline catalyst at 120-150° C. and 1-30 p.s.i.g. until one to ten moles of the oxide is added. In place of the alkaline catalyst, acidic catalysts such as BF<sub>3</sub>, H<sub>3</sub>PO<sub>4</sub> and the like can be used. Secondary alcohols such as 2-decanol, 3-decanol, 4-decanol, 3-dodecanol, 25 4-tetradecanol, 6-hexadecanol, and the like, or their admixtures as well as alkylphenols such as octylphenol, linear decyl phenol, branched dodecylphenol, etc., can be substituted for the primary aliphatic alcohol. The resultant alkyl or alkylarylpolyalkyleneoxyalkanol is then reacted 30 with phosgene to form the corresponding alkyl or alkyl-arylpolyalkyleneoxy chlorocarbonate, and the latter compound converted to its carbamate by reaction with gamma dialkylaminopropylamine. This latter derivative is acidified and reacted with an alkylene oxide to form its quaternary 35 ammonium salt.

The new and useful antistatic agents of the present invention have been found to have unexpectedly advantageous antistatic properties, particularly when applied to synthetic fibers, such as polyesters, acrylics, polyolefins, polyamides, etc. Such antistatic agents have been found to reduce and maintain the electrostatic charges for extended periods of time below a potential of 3 kilovolts.

45 The following specific examples illustrate the new and useful product and process of the present invention. These examples are for purposes of illustration only, and the present invention is in no way to be deemed as limited thereto.

### EXAMPLE 1

50 (a) To a round bottom flask was charged a total of 288  
parts by weight of an ethoxylate (av. app. 2.0 moles EO)  
of a C<sub>12</sub>-C<sub>15</sub> straight chain primary alcohol admixture cal-  
culated as a 209 mw. average and having the composition  
55 5% C<sub>11</sub>, 25% C<sub>12</sub>, 30% C<sub>13</sub>, 30% C<sub>14</sub> and 10% C<sub>15</sub>. The  
ethoxylate was agitated at ambient temperature (20-30°  
C.) while phosgene was bubbled in under the surface over  
about 1.5 to 2.0 hours. Addition of phosgene was continued  
until examination of sample on IR showed essentially all  
60 absorption due to the hydroxyl group was eliminated. A  
total of 109 gms. phosgene (1.1 mole) were required.

(b) To a beaker equipped with agitator, two dropping funnels, thermometer and a pH meter were charged 500 ml. water and 91 gms. dimethyl propylene diamine (0.9 mole). These materials were agitated at room temperature 65 while 316 gms. of the chlorocarbonate (0.9 mole) prepared in (a) and 30% NaOH were dropped in simultaneously over about 1 to 1.5 hours at such a rate as to maintain the pH between 10.0 to 10.5. A total of 141 gms. 30% NaOH was required. After all reactants were added, the 70 batch was agitated 15 minutes at room temperature and then brought to pH 9.0 with C.P. HCl. A total of 2.0 gms. were required. The product was then stripped of water at 40 mm. pressure and the residue was filtered. The yield was 293 gms.

75 (c) To a 1 liter 4-necked flask with joints clamped for

slight pressure were charged 250 gms. (0.6 mole) of the above carbamate, 250 ml. H<sub>2</sub>O and 104 gms. C.P. HCl to bring pH to 3.0 to 3.5. Materials were agitated at 50-60° C. and purged with N<sub>2</sub>. Ethylene oxide (26 gms. from cylinder) were added. A total of 19.0 gms. were absorbed.

The product was stripped to 110° C. pot temperature under line vacuum and then filtered.

The weight of the final product was 187 gms.

Percent nitrogen ..... 4.9 10  
Theory ..... 5.6

to bring pH to 3.0 to 3.5. Materials were agitated at 50-60° C. and purged with N<sub>2</sub>. Ethylene oxide (36.5 gms. from cylinder) were added. A total of 24 gms. were absorbed.

The product was stripped to 110° C. pot temperature under line vacuum and then filtered.

The weight of the final product was 147 gms.

Percent nitrogen ..... 4.8  
Theory ..... 5.0

The product corresponded, in general, to the formula:



The product, in general, corresponds to the formula:



(d) The quaternary formed above was applied from MeOH/CCl<sub>4</sub> (520 mls./1000 mls.) solvent mixture to polypropylene and Dacron swatches at 1.25% application rate according to AATCC Standard Test Method 76-1959.

The swatches were conditioned at 72° F. and 50% relative humidity for at least 24 hours and the resistivity measured. Results were as follows:

|                           | Log ohms/square |        |
|---------------------------|-----------------|--------|
|                           | Polypropylene   | Dacron |
| Control.....              | 14.64           | 13.26  |
| Quaternary carbamate..... | 7.77            | 7.65   |

## EXAMPLE II

Parts (a) and (b) were the same as in Example I.

(c) To a 1 liter 4-necked flask with joints clamped for slight pressure were charged 250 gms. (0.6 mole) of the above carbamate, 250 ml. H<sub>2</sub>O and 108 gms. 1/1 H<sub>2</sub>O/C.P. NH<sub>3</sub> to bring pH to 3.0 to 3.5. Materials were agitated at 50-60° C. and purged with N<sub>2</sub>. Ethylene oxide (36 gms. from cylinder) were added. A total of 19.5 gms. were absorbed.

The product was stripped to 110° C. pot temperature under line vacuum and then filtered.

The weight of the final product was 242 gms.

Percent Nitrogen ..... 7.2 50  
Theory ..... 8.0

The products correspond, in general, to the formula



(d) The quaternary formed above was applied from MeOH/CCl<sub>4</sub> (520 mls./1000 mls.) solvent mixture to Dacron and to cotton swatches at 1.25% application rate according to AATCC Standard Test Method 76-1959.

The swatches were conditioned at 72° F. and 50% relative humidity for at least 24 hours and the resistivity measured. Results were as follows:

|                           | Log ohms/square |        |
|---------------------------|-----------------|--------|
|                           | Dacron          | Cotton |
| Control.....              | 13.26           | 14.24  |
| Quaternary carbamate..... | 7.59            | 7.90   |

## EXAMPLE III

Parts (a) and (b) were the same as in Example I.

(c) To a 1 liter 4-necked flask with joints clamped for slight pressure were charged 250 gms. (0.6 mole) of the above carbamate, 250 ml. H<sub>2</sub>O and 47.5 gms. H<sub>3</sub>PO<sub>4</sub> 75

to bring pH to 3.0 to 3.5. Materials were agitated at 50-60° C. and purged with N<sub>2</sub>. Ethylene oxide (36.5 gms. from cylinder) were added. A total of 24 gms. were absorbed.

The product was stripped to 110° C. pot temperature under line vacuum and then filtered.

The weight of the final product was 190 gms.

Percent nitrogen ..... 5.9  
Theory ..... 6.3

The product corresponded, in general, to the formula:



(d) The quaternary formed above was applied from MeOH/CCl<sub>4</sub> (520 mls./1000 mls.) solvent mixture to Nylon Faile and polypropylene swatches at 1.25% application rate according to AATCC Standard Test Method 76-1959.

The swatches were conditioned at 72° F. and 50% relative humidity for at least 24 hours and the resistivity measured. Results were as follows:

|                           | Log ohms/square |               |
|---------------------------|-----------------|---------------|
|                           | Nylon faile     | Polypropylene |
| Control.....              | 13.91           | 14.64         |
| Quaternary carbamate..... | 7.85            | 7.80          |

## EXAMPLE IV

(a) To a round bottom flask was charged a total of 174 parts by weight of an ethoxylate (1.0 mole E.O.) of octyl alcohol. The ethoxylate was agitated at ambient temperature (20-30° C.) while phosgene was bubbled in under the surface over about 1.5 to 2.0 hours. Addition of phosgene was continued until examination of sample on IR showed essentially all absorption due to the hydroxyl group was eliminated. A total of 107 gms. phosgene (1.08 mole) were required.

(b) To a beaker equipped with agitator, two dropping funnels, thermometer and a pH meter were charged 300 ml. water and 91 gms. dimethyl propylene diamine (0.9 mole). These materials were agitated at room temperature while 213 gms. of the chlorocarbonate (0.9 mole) prepared in (a) and 30% NaOH were dropped in simultaneously over about 1 to 1.5 hours at such a rate as to maintain the pH between 10.0 to 10.5. A total of 38 gms. 30% NaOH was required. After all reactants were added, the batch was agitated 15 minutes at room temperature and then brought to pH 9.0 with C.P. HCl. A total of 3.0 gms. were required. The product was then stripped of water at 40 mm. pressure and the residue was filtered. The yield was 218 gms. Theoretical yield was

$$0.9 \times 303 = 272 \text{ gms.}$$

so the percent yield was 80.2.

(c) To a 1 liter 4-necked flask with joints clamped for a slight pressure were charged 182 gms. (0.6 mole) of the above carbamate, 175 ml. H<sub>2</sub>O and 45 gms. H<sub>3</sub>PO<sub>4</sub> to bring pH to 3.0 to 3.5. Materials were agitated at 50-60° C. and purged with N<sub>2</sub>. Ethylene oxide (33 gms. from cylinder) were added. A total of 21 gms. were absorbed.

The product was stripped to 110° C. pot temperature under line vacuum and then filtered.

The weight of the final product was 190 gms.

Percent nitrogen ..... 5.9  
Theory ..... 6.3

The product conforms, in general, to the formula:



(d) The quaternary formed above was applied from MeOH/CCl<sub>4</sub> (52.0 mls./1000 mls.) solvent mixture to Dacron and Nylon Faile swatches a 2.5% application rate according to AATCC Standard Test Method 76-1959.

to bring pH to 3.0 to 3.5. Materials were agitated at 50-60° C. and purged with N<sub>2</sub>. Ethylene oxide (30 gms. from cylinder) were added. A total of 22 gms. were absorbed.

5 The product was stripped to 110° C. pot temperature under line vacuum and then filtered.

The weight of the final product was 495 gms.

Percent nitrogen 2.9

Theory 3.22

10 The product corresponded, in general, to the formula



The swatches were conditioned at 72° F. and 50% relative humidity for at least 24 hours and the resistivity measured.

Results were as follows:

|                           | Log ohms/square |             |
|---------------------------|-----------------|-------------|
|                           | Dacron          | Nylon faile |
| Control.....              | 13.26           | 13.91       |
| Quaternary carbamate..... | 8.92            | 9.14        |

#### EXAMPLE V

(a) To a round bottom flask was charged a total of 660 parts by weight of an ethoxylate (10.0 moles E.O.) of nonylphenol. The ethoxylate was agitated at ambient temperature (20-30° C.) while phosgene was bubbled in under the surface over about 1.5 to 2.0 hours. Addition of phosgene was continued until examination of sample on IR showed essentially all absorption due to the hydroxyl group was eliminated. A total of 112 gms. phosgene (1.15 mole) were required.

(b) To a beaker equipped with agitator, two dropping funnels, thermometer and a pH meter were charged 1100 ml. water and 91 gms. dimethyl propylene diamine. (0.9 mole). These materials were agitated at room temperature while 650 gms. of the chlorocarbonate (0.9 mole) prepared in (a) and 30% NaOH were dropped simultaneously over about 1 to 1.5 hours at such a rate as to maintain the pH between 10.0 to 10.5. A total of 150 gms. 30% NaOH was required. After all reactants were added the batch was agitated 15 minutes at room temperature and then brought to pH 9.0 with C.P. HCl. A total of 5.0 gms. were required. The product was then stripped of water at 40 mm. pressure and the residue was filtered. The yield was 596 gms. Theoretical yield was

$$0.9 \times 789 = 710 \text{ gms.}$$

so the percent yield was 84.0.

(c) To a 1 liter 4-necked flask with joints clamped for slight pressure were charged 475 gms. (0.6 mole) of the above carbamate, 450 ml. H<sub>2</sub>O and 99 gms. C.P. HCl

20 (d) The quaternary formed above was applied from MeOH/CCl<sub>4</sub> (520 mls./1000 mls.) solvent mixture to polypropylene and Orlon swatches at 1.25% application rate according to AATCC Standard Test Method 76-1959.

The swatches were conditioned at 72° F. and the 50% relative humidity for at least 24 hours and the resistivity measured. Results were as follows:

|                           | Log ohms/square |       |
|---------------------------|-----------------|-------|
|                           | Polypropylene   | Orlon |
| Control.....              | 14.64           | 14.24 |
| Quaternary carbamate..... | 9.93            | 9.86  |

#### EXAMPLE VI

40 Baths were prepared by weighing 1.25 g.-2.50 g. of antistat into tared 4 oz. WMSC clear bottles. The solvent mixture (520 mls. methanol/1000 mls. carbon tetrachloride) was then added by volume, i.e., 99 mls. and 97 mls., respectively, to produce soluble, fluid, clear solutions in each case.

45 5 The preweighed and conditioned swatches (11×12 cms.) were immersed in the appropriate baths for one hour with good agitation. This agitation consisted of light shaking and swirling by hand. The swatches all appeared to wet nicely and uniformly. Removed swatches and allowed to 50 drain back into bottle for about ten seconds, then hung under balance on a hook and adjusted to 100% pickup by lightly blotting with paper towels. All swatches were relatively easy to adjust to 100% pickup.

The finished swatches were then placed in the steam heated cabinet overnight at 50° C. before conditioning.

55 After a minimum of 40 hours conditioning at 50% R.H. and 73° F., the resistance of each swatch was measured front and back across the warp. The average of these two readings on each swatch was then calculated to obtain log ohms/square that is recorded in the following table:

#### LOG OHMS/SQUARE

| Composition applied        | Percent application bath | Nylon faile | Polypropylene | Dacron type 54 | Orlon (T-42) |
|----------------------------|--------------------------|-------------|---------------|----------------|--------------|
| Product Ex. I.....         | 1.25                     | 8.18        | 7.77          | 7.65           | 8.10         |
|                            | 2.50                     | 7.90        | 7.43          | 7.45           | 7.73         |
| Product Ex. II.....        | 1.25                     | 8.15        | 7.84          | 7.59           | 7.90         |
|                            | 2.50                     | 7.69        | 7.62          | 7.41           | 7.78         |
| Product Ex. III.....       | 1.25                     | 7.85        | 7.80          | 7.52           | 8.05         |
|                            | 2.50                     | 7.75        | 7.49          | 7.21           | 7.62         |
| Catanae <sup>1</sup> ..... | 1.25                     | 7.49        | 8.56          | 7.16           | 8.19         |
|                            | 2.50                     | 8.33        | 8.27          | 7.99           | 8.27         |
| Control.....               |                          | 13.91       | 14.64         | 13.26          | 14.24        |

<sup>1</sup> Commercial antistatic agent of cationic type.

**9**  
**EXAMPLE VII**

Samples of the product of Example III were submitted for resistivity measurements. The first sample was approximately 60% active in the mixture of isopropanol and water in which it was prepared while solvents had been stripped from the second sample, and it was essentially 100% active.

The samples were applied at the 1.25% level from isopropanol solutions in 4 oz. WMS bottles to Nylon Faile, polypropylene, Dacron (Type 54), and Orlon (T-42) fabrics. These isopropanol solutions were slightly hazy, so repeat applications were made from solutions containing 70 g. isopropanol and 30 g. water. The products were completely soluble in this mixture, giving clear solutions.

The samples were adjusted to 100% wet pick-up, dried in the steam cabinet overnight, and then conditioned at 73° F. and 50% R.H. for measurement of resistivity. The absolute pickup was measured by weighing the con-

**10**

$R_3$  is a hydroxyalkyl radical having from 1 to 4 carbon atoms; and  
Y is an anion.

2. An antistatic compound of the formula:



3. An antistatic compound of the formula:



15 4. An antistatic compound of the formula:



5. An antistatic compound of the formula:



6. An antistatic compound of the formula:



ditioned swatches before and after treatment. The data are recorded in the following table.

| Concentration in application bath, percent         | Nylon fail              |              | Polypropylene           |              | Dacron (type 54)        |              | Orlon (T-42)            |              |
|----------------------------------------------------|-------------------------|--------------|-------------------------|--------------|-------------------------|--------------|-------------------------|--------------|
|                                                    | Percent by wt. on fiber | Log ohms/sq. | Percent by wt. on fiber | Log ohms/sq. | Percent by wt. on fiber | Log ohms/sq. | Percent by wt. on fiber | Log ohms/sq. |
| <b>Applied from isopropanol:</b>                   |                         |              |                         |              |                         |              |                         |              |
| 1.25                                               | 1.25                    | 8.94         | 1.04                    | 8.61         | 1.28                    | 8.69         | 1.27                    | 9.16         |
| 1.25                                               | 1.31                    | 8.97         | 1.09                    | 8.71         | 1.21                    | 8.72         | 1.16                    | 9.15         |
| <b>Applied from 70 isopropanol/30 water blend:</b> |                         |              |                         |              |                         |              |                         |              |
| 1.25                                               | 1.05                    | 9.43         | 1.21                    | 8.87         | 1.07                    | 9.00         | 0.91                    | 9.42         |
| 1.25                                               | 0.80                    | 9.63         | 0.84                    | 8.98         | 0.97                    | 8.90         | 1.10                    | 9.45         |
|                                                    |                         | 14.04        |                         | 14.13        |                         | 13.44        |                         | 14.13        |

While certain preferred embodiments of the present invention have been shown by way of specific example, it is to be understood that the present invention is in no way to be deemed as limited thereto but should be construed as broadly as all or any equivalents thereof.

What is claimed is:

1. An antistatic compound of the formula:



wherein:

R is a radical selected from alkyl and alkyaryl radicals having at least 7 carbon atoms;

X is selected from hydrogen, methyl or ethyl;

n is a number from 1 to 10;

$R_1$  and  $R_2$  are selected from alkyl and hydroxyl alkyl radicals having from 1 to 3 carbon atoms;

**References Cited**  
**UNITED STATES PATENTS**

2,626,876 1/1953 Carnes ----- 117—138.8  
2,721,208 10/1955 Lossee et al. ----- 260—482 XR  
55 2,998,445 8/1961 Stewart et al. ----- 260—482  
3,359,303 12/1967 Coker et al. ----- 260—482

LORRAINE A. WEINBERGER, Primary Examiner.  
A. P. HALLUIN, Assistant Examiner.

U.S. Cl. X.R.

117—138.8, 139.5; 260—75, 93.7, 94.9